

May 14, 1940.

A. P. MEYER

**2,200,717**

## PROCESS FOR COKING PITCH

Filed Aug. 17, 1938

2 Sheets-Sheet 1



Inventor

Albert P. Meyer,

By K. P. McElroy

Attorney

May 14, 1940.

**A. P. MEYER**

**2,200,717**

## PROCESS FOR COKING PITCH

Filed Aug. 17, 1938

2 Sheets-Sheet 2



Turing. 3.

Inventor  
*Albert P. Meyer,*

K. P. McElroy

Attorney

## UNITED STATES PATENT OFFICE

2,200,717

## PROCESS OF COKING PITCH

Albert P. Meyer, Pittsburgh, Pa., assignor to  
 Pittsburgh Coke & Iron Company, Pittsburgh,  
 Pa., a corporation of Pennsylvania

Application August 17, 1938, Serial No. 225,438

2 Claims. (Cl. 202—19)

This invention relates to coking pitch; and it comprises a method of making substantially pure hydrogen-free carbon in friable form suitable for electrode use wherein a body of molten coal tar pitch is established as a long narrow pool not over 30 inches in width and is subjected to destructive distillation by the action of hot gaseous products of combustion passing upwardly therethrough until the residual content of volatile matter is removed and until the liquid pitch changes to a loose, spongy, vesicular body of carbon and shrinks away from the walls of the containing chamber, and continuing passage of the hot combustion products in contact with the body until a carbon is obtained containing not more than 1 per cent volatile matter (hydrocarbons); all as more fully hereinafter set forth and as claimed.

The present invention is directed to making a pure carbon suitable for electrodes, a product which is as nearly pure C as possible, with the least amount of manipulation and apparatus. In carbon for the manufacture of electrodes an extremely low content of volatile matter, that is, of carbon compounds containing hydrogen, is desirable; a volatile matter content of 1 per cent or less. On the other hand the mechanical strength and the type of cell structure necessary in coke to be used for metallurgical purposes (as in a cupola or blast furnace), are not required or desired. In a carbon to be comminuted and reshaped as electrodes, high mechanical strength is not so desirable as a friable, readily comminuted preparation.

In the present invention coal tar pitch is used as the immediate source material for pure carbon; pitch being the residue in the distillation of tar for recovery of coal tar oils, light and heavy, cresols, creosote, etc. The pitch can be obtained as the residue from ordinary distillation of tar in any of the usual ways; or if desired the pitch can be produced from tar in the same apparatus later used for carbonizing the pitch, in continuous successive operations. In another and companion application Ser. No. 225,439 I have described and claimed a method in which both distillation and carbonization are successively effected in the same apparatus.

Coal tar in its original state contains a considerable amount of volatile hydrocarbons distillable as such, which are commercially worth while. These may be removed and recovered by heating the tar to a temperature of the order of 500° to 700° F., the residue being reduced to hard pitch. Pitch at a temperature of this order is

utilized in the present invention. Further application of heat to the pitch effects destructive distillation. As a matter of fact, simple distillation and destructive distillation overlap, but the distillation which occurs at temperatures lower than the aforesaid range of temperatures in the ordinary types of tar still is predominantly simple distillation, while that occurring at higher temperatures is predominantly destructive distillation. Up to a certain point distillation is endothermic, but as the temperature of the pitch rises to some point above 1000° F. with destructive distillation, the material passes through a definitely exothermic stage and a "self-coking" effect is noticeable.

I have observed that processes of this character in which destructive distillation and coking occur ordinarily yield a product which is more aptly described as a "semi-coke" than as a true coke; a material having a definite cell structure but containing a substantial content of volatile matter, usually in excess of 3 per cent. Carbonization has not been completed. I find that for my purposes in order to complete carbonization and destructive distillation, with removal of volatile matter down to 1 per cent or less in the final product, finishing temperatures substantially in excess of 1500° F., and preferably of the order of 1800° F., are required. At such temperatures all of the hydrocarbons present tend to break down to free carbon and hydrogen. The action in this final stage is neither markedly endothermic nor exothermic, but it does require application of sufficient heat to maintain temperatures of the order noted for sufficient time to complete the action; that is, a soaking heat to insure that all portions of the mass of residue are subjected to such temperatures. However, if the carbonaceous mass is disposed in such fashion that the center of the mass is located at a considerable distance from the point of application of heat, it is impossible as a practical matter to reduce the average volatile matter content of the mass to a sufficiently low point, even when the walls of the retort are maintained at the aforesaid high temperature.

A number of processes have been proposed and utilized in the past for making coke from coal tar; mostly for metallurgical purposes. For the manufacture of low volatile carbon for electrodes from coal tar pitch, these leave much to be desired. Some of these processes utilize coking ovens similar or identical to those designed for the manufacture of high temperature by-product coke from coal. As a practical matter, these ovens are extremely expensive, and

serious difficulties are encountered in their use, when attempting to coke pitch, principally due to foaming during the coking operation. All attempts to overcome these difficulties result, in one way or another, in reducing the efficiency of the operation from other standpoints. In the present process final conversion of the pitch into an open textured puffed up solidified mass is desired and this foaming effect is utilized.

10 Among the objects achieved by my invention is the provision of a process for reducing coal tar pitch to electrode carbon containing 1 per cent volatile matter or less, in a unitary operation, with a minimum of mechanical difficulties, 15 with high yields of products, and in a reasonably short operating period.

Additional operative advantages and improvements obtained in accordance with my invention will also be evident from the following description.

20 The carbonizing apparatus employed in my invention comprises a refractory structure so constructed as to provide a retort chamber elongated vertically and in one horizontal direction, while 25 the other horizontal dimension of the oven is restricted to 30 inches or less. Thus, typically suitable dimensions for a retort to be used in the performance of my carbonizing process are: from 16 to 24 inches wide; from 8 to 16 feet high; and 30 from 8 to 20 feet long. Of these dimensions, the length is the least important. The chamber is provided with vertical doors at each end, for pushing the finished coke horizontally out of the oven in a manner similar to the manner in which 35 coke is removed from by-product coke ovens operating on coal. Each chamber is provided with a plurality of inlets near the floor thereof, for introducing hot gases, which in the ordinary instance will comprise gases produced by the combustion 40 of solid, liquid or gaseous fuel. Means are provided for leading the exit gases and vapors to suitable condensers, heat exchangers, coolers, and the like, and ultimately to an exhaust fan capable of maintaining a substantial vacuum.

45 In the operation of the apparatus, coal tar pitch is introduced into the retort chamber in sufficient amount to fill the chamber to about one-third to one-half of its capacity, that is, to a depth between 3 and 8 feet. The pitch is introduced in a fluid or molten condition, and preferably at a temperature of from 500° to 700° F. The pitch may be introduced at a lower temperature in some cases, but in such event the oven should be preheated in order to avoid chilling 55 the mass of pitch to a solid state. If desired the pitch can be produced in situ by distillation of tar in the retort chamber, as described below. Hot gases of combustion, as free of oxygen as possible, are then bubbled through the liquid 60 charge under a vacuum. These gases not only serve to supply heat but also cause free evaporation and, under the influence of the applied vacuum, effectively cause the entire mass of the charge to be subjected to pressures below atmospheric. The gases reaching the upper level 65 of the charge, together with vapors of volatile matter evaporated thereby, or produced by destructive distillation of the charge, are passed through a condenser of suitable type. Oils thus 70 condensed are valuable as by-products. The cooled gases then pass from the condenser to an exhaust fan operated to create a rather high suction; say, about 14 inches (water) at the top of the charge in the oven.

75 During the initial stage of the carbonizing op-

eration, the heating gases may be supplied at a temperature of the order of 1400° to 1600° F. But in any event, the temperature of the heating gases should be gradually increased to around 1800° F. Destructive distillation begins almost 8 immediately and the temperature of the charge rises rapidly to a point usually a little above 1100° F. At this point there is usually a sudden drop in temperature to around 1000° F. and there appears to be a "change of phase" in the mass of 10 the material being carbonized; at this point the transition from a body of liquid to a more or less solid material occurs.

Immediately following the comparatively small drop in temperature mentioned there is ordinarily a very sharp rise in temperature, due to exothermic reaction. This rise is so marked that in some cases the temperature of the charge may actually exceed that of the heating gases. At this point the charge tends to be quite reactive 20 with oxygen and it is especially desirable to control the amount of oxygen in the heating gases very closely, in order to prevent loss of material through oxidation or combustion. In any event, the flow of hot gases is continued until the entire 25 mass of the charge is brought to a temperature substantially in excess of 1500° F., and preferably of the order of 1800° F., and until the average amount of volatile matter in the charge is reduced to 1 per cent or less.

With a charge not more than 30 inches thick, the time required for this portion of the operation is not excessive, and due to the fact that the coke is of cellular and porous structure, there is an effective penetration of heat throughout the 30 mass, although a considerable portion of the hot gases at this stage undoubtedly flows between the carbonaceous mass and the vertical walls of the oven. In fact, in some cases the exothermic action which takes place after the "change of 35 phase" referred to above is so marked, and the temperature of the charge rises so rapidly to a high point that the finishing or calcining period can be reduced to a minimum of around thirty 40 minutes. The amount of gas necessary to pass 45 through the retort at this stage is not excessive, and there is little or no condensable vapor in the exit gases. Consequently, it is unnecessary to pass the exit gases at this stage of the operation 50 through the condenser used during the earlier 55 stages; these exit gases may conveniently be employed for preheating another retort of the same type, or for preheating the charge or the fuel or air used in producing the gases of combustion, or they may be employed for the purpose of distilling coal tar to pitch suitable for charging into the operation.

I have found that, in a retort of the character indicated, wherein carbonization is effected by supplying hot gases directly to the mass of pitch 60 being coked, the foaming difficulties encountered in most pitch coking operations are avoided, presumably because the convective distillation effect of these gases causes constituents which would otherwise cause foaming to be removed more or 65 less gradually instead of being liberated during a comparatively short period. However, during the destructive distillation the charge usually puffs up to some extent and becomes for a time a more or less vesicular doughy mass, usually exceeding the volume of the original pitch charge. As the operation progresses farther and the volatile matter of the final product falls to 1 per cent or less, shrinkage takes place, the final volume 70 of the charge being ordinarily about equal to or 75

somewhat less than that of the original liquid pitch charge.

After the operation has been completed, the flow of gases is discontinued, the doors at the ends of the retorts are removed, and the coke is discharged from the oven or retort by pushing it horizontally with apparatus designed for that purpose. The doors are then replaced, and, where necessary, after preheating to around 500° to 700° F., the oven is then ready to receive a fresh charge and the operation is repeated.

The following description, given in conjunction with the drawings illustrating and forming part of this specification, will serve to explain and exemplify my invention in further detail. In these drawings,

Fig. 1 is a vertical cross-sectional view of a coke oven suitable for use in my invention;

Fig. 2 is a horizontal sectional view of the same oven taken along the lines 2—2 of Fig. 1; and

Fig. 3 is a more or less diagrammatic view of the oven shown in Figs. 1 and 2, in association with auxiliary apparatus employed in carrying out the process of my invention.

Similar reference numerals designate similar parts in the several views of the drawings.

As shown in Figs. 1, 2 and 3, I provide a coking retort oven comprising a refractory structure 10 so constituted as to provide a retort space of rectangular shape, having vertically disposed doors 11 at the ends thereof and suitable supporting framework 12. As has been indicated hereinabove, the dimensions of the retort space within the refractory structure 10 may vary to some extent, but the retort illustrated in the drawings is one having internal dimensions as follows: length, 8 feet; height, 10 feet; width (at discharge end), 20 inches; width (at pusher end), 16 inches. A series of conduits or tuyères 13 is provided in the bottom portion of each of the vertical walls of the structure 10, for admitting gases of combustion. As shown in the drawings, the tuyères in one of the vertical walls are preferably staggered with respect to the tuyères in the opposite wall; each tuyère lies opposite to a point about midway between adjacent tuyères in the opposite wall. The tuyères 13 are in turn connected to horizontal flues 14 in such a manner as to provide for easy access and cleaning of the tuyères 13. The flues 14 are in turn connected through vertical risers 15 to a flue manifold structure 16 which is supplied with hot gaseous products of combustion through a conduit 17 from a combustion chamber 18 having a fuel burner 19. All of these conduits and tuyères are lined with refractory material for protection.

Liquefied pitch, preferably at a temperature of 500° to 700° F., is introduced into the retort through a line 20 having a valve 21 and communicating with a source of supply (not shown) of the charge, such as a tar still. Or if desired the pitch can be produced directly in the retort by distillation of tar, as described below.

At the top of each retort there is provided one or more off-take flues 22 having a removable cap or stack valve 23 and communicating through a crossover flue 24 and a down-comer 25 to a tar trap 26 having a drain 27.

From the tar trap 26 the gases and vapors from the interior of the retort pass through a pipe or flue 29 into a scrubber 30, the interior of which is provided with tile packing 31 or other suitable gas-and-liquid-contact material. Condensate withdrawn from the bottom of the scrubber 30 is withdrawn therefrom through a valved

pipe 32 leading to a pump 33. A portion of this condensate is recirculated through a line 34, an indirect cooler 35 and a line 36 to a spray or other distributing device 37 located in the top of the scrubber 30. Another portion is pumped through 5 a branch line 38 into the down-comer 25. Excess condensate is removed through a valved line 39 and sent to storage.

The cooled gases leaving the scrubber 30 pass through a conduit 40 to an exhaust or vacuum 10 pump 41 which in turn delivers them through a conduit 42 to an exhaust stack 43 or, where desired, into suitable heat exchangers or preheating devices. Any excess liquid collecting in the bottom of the exhaust stack 43 is removed through 15 a line 44 and passes to a suitable storage vessel 45. I also provide a valved line 46 for introducing a portion of the condensate into the conduit 40.

The operation of this apparatus will be clear 20 from the description given hereinabove, pitch being charged into the retort structure 10 and heated internally by means of hot gases produced in the combustion chamber 18, and the temperature of the gases being regulated in accordance 25 with the foregoing description.

After the operation has been completed, and the charge is reduced to the desired low volatile content, the doors 11 at the ends of the retort structure are removed, and the coke is pushed 30 out of the oven by means of a pusher 50, similar to those used in connection with by-product coke ovens commonly used for coking coal.

Where desired, a plurality of retorts similar 35 to those described and illustrated hereinabove may be employed, it being preferable to build these in the form of a battery of retorts. In such case provision is, of course, made for operating the retorts alternately or in a series of scheduled operations, and for connecting and disconnecting 40 the exhaustor 41 to such oven or ovens as may be in operation at any given time.

As stated, if desired the pitch can be made in situ from coal tar, tar being introduced into chamber 10 through conduit 20 in amount sufficient to fill the chamber about two-thirds full. The tar is heated by means of hot gases from the combustion chamber 18. Distillation takes place and the distillate is condensed in tar trap 26 and scrubber 30. In due course the tar becomes converted into pitch and the pitch is then carbonized 50 by destructive distillation in the procedure explained above.

While my invention has been described hereinabove with reference to various illustrative details of apparatus and operation, it will be understood by those skilled in the art that my invention in its broadest aspects is not limited to such details but may be variously practiced and embodied within the scope of the claims herein- 55 after made.

What I claim is:

1. In the destructive distillation and carbonization of coal tar pitch by hot combustion gases, an improved process of making substantially 65 pure carbon which comprises establishing a horizontally elongated substantially rectangular body of molten pitch not over 30 inches in width, introducing gaseous products of combustion entering at a temperature of 1400°-1600° F. into 70 said body at a plurality of points along its length and near the bottom thereof while maintaining a partial vacuum thereabove, gradually raising the temperature of the combustion gases to about 1800° F. until the pitch body becomes a vesicular 75

solid residue and continuing a flow of the hot gases through and in contact with the solid residue until it reaches a temperature exceeding 1500° F. and solid carbon is produced having a 5 volatile matter content less than 1 per cent by weight.

2. A method of making substantially pure carbon from coal tar pitch which comprises establishing a horizontally and vertically elongated body of molten pitch not over 30 inches in width, 10 introducing gaseous products of combustion entering at a temperature of 1400° to 1600° F. into

said body at a plurality of points along its length near the bottom thereof while maintaining a partial vacuum thereabove, gradually raising the temperature of the combustion gases until the pitch body becomes a vesicular residue and continuing a flow of hot gases along and in contact with the solid residue until it reaches a temperature exceeding 1500° F. and solid carbon is produced having a volatile matter content less than 1 per cent by weight. 5

ALBERT P. MEYER.